

Dec. 22, 1959

J. J. KELLEY

2,918,389

PROTECTIVE COVERING FOR METALS

Filed Feb. 2, 1956

3 Sheets-Sheet 1



FIG. 1.



FIG. 2.

INVENTOR.  
JOHN J. KELLEY  
BY  
*J. J. Kelley*  
ATTORNEY

Dec. 22, 1959

J. J. KELLEY

2,918,389

PROTECTIVE COVERING FOR METALS

Filed Feb. 2, 1956

3 Sheets-Sheet 2



FIG. 3.

INVENTOR.  
JOHN J. KELLEY  
BY  
*John J. Kelley*  
ATTORNEY

Dec. 22, 1959

J. J. KELLEY

2,918,389

PROTECTIVE COVERING FOR METALS

Filed Feb. 2, 1956

3 Sheets-Sheet 3



FIG. 4.

INVENTOR.  
JOHN J. KELLEY  
BY  
*C. M. Springer*  
ATTORNEY

# United States Patent Office

2,918,389

Patented Dec. 22, 1959

1

2,918,389

## PROTECTIVE COVERING FOR METALS

John J. Kelley, Golden, Colo.

Application February 2, 1956, Serial No. 563,171

2 Claims. (Cl. 117—68)

This invention relates to a material or composition for use on metallic structures that are exposed to severe corrosive conditions.

After study of the processes of corrosion, it has been determined that it would be advantageous to provide in a single wrapping material a mechanical shield, an electrical insulator and a chemical protector. The mechanical shield must be of sufficient physical strength to resist abrasion, frictional wear and soil stresses when the protective material is to be buried underground. Further, the shield must be resistant to the ingress of moisture and, insofar as possible, the dissolving action of crude oil or crude oil products that might saturate the soil.

While the mechanical shield should be designed to resist the physical forces that act to deteriorate the protective material, it is advantageous to provide a second barrier of protection that may be embodied in the same composition or material. The second, or insulator barrier, should be designed to prevent corrosion due to the co-action of electrolytic cells in the surface of the metal and electrical currents in the structure itself or stray electric currents in the surrounding soil when buried underground. Accordingly, it is desirable to incorporate in the unitary protective material an electrical insulator having a high dielectric strength, so that a thin sheet or layer of the material may be used to avoid destroying the flexibility or pliability of the entire material. In addition to flexibility, which is provided to avoid cracking and peeling when the material is being applied around a pipe or other curvature of small diameter in cold weather, the electrical insulator should be of a type that is unaffected by bacteria, acids and alkalis normally present in the soil.

A third barrier of protection should be provided to avoid the effects of chemical corrosion and to act as a priming mass. For such purpose, this innermost shield should be a material having the ability to penetrate through and around an existing body of rust or mill scale to isolate all oxidation products from the base metal and to provide a protective film on the base metal, which, together with inhibitors, repels any corrosive action of the surrounding media. This innermost shield should further be possessed of properties which will prevent the rupture of the shield by abrasions and scratches. Accordingly, this chemical barrier should be of a non-drying type that will flow to cover any abrasions or tiny pock marks or depressions in the metallic surface.

It is the main object of this invention to provide a material or covering which may be placed as a unit about the exterior surface of metallic objects to successfully fulfill all of the above desirable features.

Another object of this invention is to provide these desirable features in a wrapping tape that may be conveniently handled and that is adapted to be wrapped about metallic objects to provide multiple layer abrasion and corrosion resistant properties.

Other objects of the present invention will be apparent from the following detailed description and examples of the desirable properties of this invention, and from the drawings appended hereto, in which:

2

Fig. 1 is a perspective view in partial section showing the component elements of the completed wrapping material made in accordance with this invention.

Fig. 2 is an illustration showing the completed wrapping material in roll form.

Fig. 3 is a schematic illustration showing steps in the preparation of the exterior binder shield, and

Fig. 4 is a schematic illustration showing the application of the inner priming mass to the exterior binder shield material.

Briefly stated, the present invention provides a wrapping material or coating that may be placed about metallic objects to prevent corrosion due to either mechanical abrasion, electrolytic effects or chemical decomposition.

15 In order to attain the desired result, it has been found advisable to provide the desired product in a roll, wrap or bandage from which it may be readily applied to pipe lines or other curved surfaces.

To attain the desired properties, materials of different 20 consistency are applied to opposite sides of a binder material, such as a glass fibre mat, in such manner that the exterior face of the assembled wrap will present a surface that is resistant to abrasion and that also acts as an electrolytic insulator. A priming mass made up pri-

25 marily of a petrolatum material is applied to the inner face of the bandage for intimate contact with the metallic object to be preserved. In order to decrease the moisture penetrability of the priming mass, certain additives are mixed in the petrolatum, and rust inhibitors are likewise 30 introduced to further prevent chemical or hydrolytic corrosion. In order that the bandage may be unwound for application, both the exterior surface and the priming mass possess additional physical properties that will allow the bandage to be unwound even after exposure to 35 direct sun or cool temperatures.

A specific embodiment of the present invention would be prepared in accordance with the following provisions. In order to develop a priming mass having the desired properties, it has been found that petrolatum, an amorphous mineral oil wax, is a most satisfactory base material; however, several desirable and necessary features of a satisfactory priming mass are lacking in petrolatum itself. It is necessary, for instance, to adjust the softening point of ordinary petrolatum, so that it will not only 45 withstand the intense heat of exposure to direct sun in hot summer weather, but also so that it will withstand such heat and not penetrate and destroy or damage other parts of the roll bandage thereby making application of the bandage difficult. Further, petrolatum of itself is not 50 possessed of inhibiting qualities to counteract the corrosive effects of an already wet metallic surface.

A petrolatum product obtainable on the open market which contains some of the chemical inhibitors and which has an improved softening point desirable for the present 55 purposes and which also has improved "self-healing" qualities through the use of added ingredients is marketed by the Texas Company as their #1995 Rust Proof compound made and manufactured under a patent to Harry Roden, dated April 24, 1945, bearing Patent No. 2,374,565. In order to improve the corrosion-resistant features of this base material, additional inhibitors are added in the form of chromates of sodium and potassium to compensate for the excess moisture which it is believed 60 may be encountered at the metallic surface. The two inhibitors chosen are purposely of different solubilities, so that an initial contact between moisture and inhibitor will not leach out, dissolve or otherwise remove all of the inhibitor, but will leave some inhibitor in place in the priming mass for subsequent protection.

70 The most satisfactory quantities of additional inhibitors are equal proportions of sodium and potassium and aggregating not less than 2 pounds per 100 pounds of

#1995 Rust Proof compound and not more than 3 pounds per 100 pounds of #1995 Rust Proof compound. The inhibitors should be finely pulverized and thoroughly dispersed throughout the compound for best results.

It has been found that under certain conditions it is necessary to further elevate the softening point of the #1995 Rust Proof compound. Where the roll bandage is to be used during the summer season, it is preferable to add quantities of Dylt or Dygt polyethylene resin, which is commercially available from the Bakelite Corporation. This addition is accomplished by preparing a concentrate of the #1995 compound and a quantity of Dylt or Dygt, which is thoroughly mixed before subsequent addition to the bulk #1995 compound, which has been liquefied by application of heat. The addition of 5 parts by weight Dylt or Dygt to 100 parts by weight of #1995 compound results in a softening point elevation of the compound to 175 degrees-180 degrees Fahrenheit, which is adequate for this purpose.

In order to further improve the "self-healing" properties of the #1995 compound and to further insure against corrosive action at the protected metallic surface resulting from a prolonged or permanent encounter with water which has penetrated the exterior barrier due to damage or imperfections in the application of the strip, it has been found desirable to add a quantity of Georgia clay as a filler material to the #1995 compound. Preferably, the Georgia clay is added to the #1995 compound in a ratio of 25 to 40 parts by weight of Georgia clay to 100 parts by weight of #1995 compound.

While it is recognized that Georgia clay is a type of bentonitic clay, and accordingly other types of bentonitic clay might presumably be substituted for the Georgia clay without departing from the scope of this invention, it must be recognized that the Georgia clay has certain inherent characteristics which make it a much more satisfactory filler material than other types of bentonitic clays. The proportions set forth herein are derived with full knowledge of the exact range of swelling due to the presence of bentonitic materials in the Georgia clay, and such proportions would necessarily have to be modified where other types of bentonitic clays are to be utilized.

In addition to the use of the Georgia clay to improve the self-healing qualities of the priming mass, it has been found desirable to add additional quantities of Georgia clay to the #1995 compound to reduce bleeding of the priming mass under conditions of extreme heating in hot summer sun. Although addition of 25 parts by weight of Georgia clay to the compound is adequate for the purpose of moisture occlusion, it is desirable to increase the proportion to 40 parts by weight of Georgia clay if the protective tape being made is to be used in summer heat. With the inclusion of the additional quantity of Georgia clay, bleeding and cross-interpenetration of the priming mass and exterior shield will be minimized.

Through experimentation, it has been found that a priming mass made in accordance with these specifications will fully satisfy the requirements and objects set forth.

While the desired mechanical shield and electrical insulator have previously been described as separate barriers, it has been found possible to select substances which will satisfy the requirements for both the electrical insulator and the mechanical shield and to combine them into a single major component of the strip of material. Asphalt, because of its high dielectric strength and strong physical properties, is particularly suited to this purpose. Because of the lack of tensile strength, however, it is important that a reinforcing medium be provided with the asphalt. A most satisfactory reinforcing medium which will serve as a binder for the bandage roll or tape is Owens-Corning's Type 20 Coromat, a glass fibre mat which has incorporated in it strong longitudinal reinforcing fibres.

In order to obtain the best shield possible, the natural

properties of different types of asphalt have been studied, and as a result of such study, it has been found that catalytically-blown Wyoming asphalt, commercially available as C-190 from the Huskey Refinery at Cody, Wyoming, and the same type of asphalt from the Lion Oil Company Refinery at Eldorado, Arkansas, are well suited for this purpose, and either may be used. The unusual qualities of these asphalts when used in membrane form, as to ductility, penetration, softening point, toughness or resistance to wear, are outstanding.

Because of the possibility of interpenetration of the asphalt shield in the petrolatum priming mass, which would make the roll bandage hard to apply, it is advantageous to harden the asphalt shield and further raise its softening point. This may best be accomplished by the addition of a high melt hydrocarbon, preferably derived from the same crude as the asphalt. One successful method has been to add #310 "Mineral Rubber" hydrocarbon pellets from the Huskey Refinery to their C-190 asphalt in a ratio of 1 part #310 to 10 parts C-190 thereby raising the softening point to 220 degrees Fahrenheit. This increase in softening point temperature is accompanied by some loss of penetration and ductility. While the foregoing proportion is satisfactory for winter use, it has been found that the ratio should be increased to 2 parts #310 to 10 parts C-190 for summer use.

To compensate for the aforementioned loss of ductility and penetration, and further to improve such qualities as impact resistance, elasticity, toughness and aging, it is advantageous to add to the asphalt a commercially available material made by Rubarite, Inc. The material used, which is a free-flowing, unvulcanized, synthetic rubber product sold under the trade name "Rubarite," is added to the asphalt in the amount of 12 parts by weight of Rubarite to 200 parts by weight of the asphalt.

As a further additive to the asphalt shield, it has been found desirable to include approximately 10 to 15 parts by weight of Georgia clay to 100 parts by weight of the asphalt to further prevent the penetration of moisture.

As a possible substitute for the glass fibre mat and asphalt exterior shield, it has been found that coal tar saturated asbestos pipe line felt, which is readily available in either 8-pound or 15-pound per 100 sq. ft. grades, may be used without further modification or change. This type material is especially useful in applications where the possibility of contact with crude oil or petroleum products is prevalent. Likewise, the material is relatively impervious to chemical solutions encountered in soil.

In order to attain the desired separation between the exterior shield material and the interior priming mass, it has been found desirable to manufacture the protective wrapping material in a batch-type step process illustrated in Figs. 3 and 4. When asphalt is to be used, the ingredients of C-190 asphalt and #310 hydrocarbon are placed together in an open-top, heated vessel and are heated to a temperature of 325 degrees Fahrenheit. The Rubarite and Georgia clay are added, and the mixture is agitated vigorously for at least 15 minutes. Thereafter, moderate agitation is continued to prevent settling out of any ingredients. The tank is equipped with a horizontal depressing rod under which the fibre glass mat is passed to insure complete saturation with the asphaltic compound. The saturated glass is then passed between two horizontal, heated tubes which serve as screeds to squeeze entrapped air out of the asphaltic compound and adjust the thickness of the reinforced asphaltic sheet to 0.031 inch, while also giving the asphaltic compound the maximum density. The sheet is then passed through a cooling chamber where it is air-cooled to about 90 degrees to 100 degrees Fahrenheit. Next, it enters a dusting chamber where it passes through an atmosphere of dust-laden air. The dust used is Georgia clay, which clings to the asphaltic sheet and especially settles in surface pores that might later be weak spots in the sheeting.

thus concentrating the swelling agent where it will be most needed, as well as reducing the sticky quality of the sheet. This feature is advantageous in reducing unwinding problems.

Meanwhile, a batch of priming mass is prepared by first preparing a concentrate of #1995 Rust Proof compound and the required amount of Dylt or Dygt. Later this concentrate is introduced into the bulk of #1995 compound, which has previously been liquified by the application of heat. In similar manner, the other ingredients, inclusive of additional inhibitor and Georgia clay, are added to the liquified mass and stirred therein to assure a complete and homogeneous mixture of all the ingredients. When thoroughly mixed, the priming mass is introduced into an open-top heated tank where it is heated to 185 degrees Fahrenheit and subjected to further agitation to prevent settling out of ingredients. This tank is equipped with a "licking" drum which is a large diameter, cylindrical drum placed in horizontal position and revolved slowly in the liquid batch of priming mass, with the upper section of the drum above the surface of the liquid mass. One satisfactory arrangement is to use a 14-inch diameter drum 37 inches long, revolving at nine revolutions per minute. The direction of rotation should be opposite to the direction of movement of the sheet.

At this point, the aforementioned pipe line felt may be substituted for the asphaltic sheet derived in the first step of this process. The sheet of desired material is then passed over the top of the drum in such manner as to cause the priming mass to be "licked" on the underneath side of the sheet. The thickness of coating applied here should be not less than  $\frac{1}{64}$  inch and not more than  $\frac{1}{32}$  inch thick. Adjustment of the thickness can be made by changing the temperature of the liquid mass, the temperature of the asphaltic or pipe line felt sheet, the speed of revolution of the drum and the speed of travel of sheet substance.

The resulting strip of material is then passed through another cooling chamber where it is reduced to atmospheric temperature or lower by air cooling. The cooled strip may then be passed through a slitting device to cut it to appropriate width before rolling, or it may be rolled in the full width of material processed to be cut later with a band saw. Another, and most desirable, method is to start the process with fibre mat or felt which has already been cut to the appropriate width.

As an example of the proportionate quantities of materials utilized in making the desired protective material, a recap of proportions is presented herewith:

100 pounds catalytically-blown asphalt-Huskey C-190.  
10 to 20 pounds #310—Huskey Co. hydrocarbon pellets.

These ingredients are added together and heated to 325° F. in an open vat. Subsequently, add:

12 pounds Rubarite—unvulcanized synthetic rubber by Rubarite, Inc.  
10 to 15 pounds Georgia clay.

Agitate the combined mixture vigorously for at least 15 minutes before passing the Type 20 glass fibre "Coromat" through the liquid mass of materials.

After the mechanical shield-insulator, as above, has cooled, it should be dusted with Georgia clay before being passed through a batch of priming mass prepared in the following proportions:

100 pounds #1995 Rust Proof compound (by The Texas Co.)  
5 pounds Dylt or Dygt polyethylene resin (by Bakelite Corp.)  
1 to 1½ pounds of sodium chromate  
1 to 1½ pounds of potassium chromate  
25 to 40 pounds Georgia clay

Insofar as it has been possible to determine, it is believed that the ingredients of #1995 Rust Proof compound made by The Texas Company come within the scope of the claims in the Roden Patent No. 2,374,565, which would indicate that the composition itself is made up of materials in the following percentages:

|                                                        | Percent |
|--------------------------------------------------------|---------|
| Petrolatum (140-150° F.M.P.)                           | 50-70   |
| Petrolatum (150-165° F.M.P.)                           | 0-15    |
| Cylinder stock                                         | 10-25   |
| Viscous pale oil                                       | 5-15    |
| Wool fat                                               | 1-8     |
| Heavy metal salt of a high molecular weight fatty acid | 0.4-1.0 |
| Alkyl ester of a high molecular weight fatty acid      | 1-5     |
| Corrosion inhibitor                                    | 0.5-2.0 |

It will be apparent from the foregoing description that the present invention is adaptable to various modifications and changes without departure from the scope of the invention as defined in the hereunto appended claims.

What is claimed is:

1. A protective covering material adapted for shipment and handling in roll bandage unit form comprising an exterior mechanical shield and electrical insulator and an interior priming mass integrally formed and applied to prevent corrosion of metallic objects, said mechanical shield and insulator comprising a glass fibre binder material and a compound for impregnating said binder, said compound comprising a base of catalytically-blown asphalt, a high melting point hydrocarbon hardener derived from the same asphalt as said base added in the ratio of 10 to 20 pounds of said hardener for every 100 pounds of said asphalt base for raising the softening point of said asphalt, and 10 to 15 pounds of Georgia clay for each 100 pounds of said base asphalt to prevent moisture penetration of said compound and exterior shield, said interior priming mass being deposited on said exterior shield for intimate contact with the metallic objects to be protected, said priming mass comprising a homogeneous mixture of materials compounded within the limits of the following proportions:

|    |                              |                                           |
|----|------------------------------|-------------------------------------------|
| 45 | Petrolatum primer            | 100 pounds.                               |
|    | Sodium chromate inhibitor    | 1 to 1½ pounds per 100 pounds of primer.  |
|    | Potassium chromate inhibitor | 1 to 1½ pounds per 100 pounds of primer.  |
| 50 | Georgia clay                 | 25 to 40 pounds per 100 pounds of primer. |

said priming mass being deposited on one side of said impregnated binder for contact with objects to be protected.

2. A protective covering material adapted for shipment and handling in roll bandage unit form comprising an exterior mechanical shield and electrical insulator and an interior priming mass integrally formed and applied to prevent corrosion of metallic objects, said mechanical shield and insulator comprising a glass fibre binder material and a compound for impregnating said binder, said compound comprising a base of catalytically-blown asphalt, a high melting point hydrocarbon hardener derived from the same asphalt as said base added in the ratio of 10 to 20 pounds of said hardener for every 100 pounds of said asphalt base for raising the softening point of said asphalt, 10 to 15 pounds of Georgia clay for each 100 pounds of said base asphalt to prevent moisture penetration of said compound and exterior shield and 6 pounds of an unvulcanized synthetic rubber compound for each 100 pounds of asphalt base to improve the ductility of said binder, said interior priming mass being deposited on said exterior shield for intimate contact with the metallic objects to be protected, said priming mass com-

prising a homogeneous mixture of materials compounded within the limits of the following proportions:

|                              |                                              |
|------------------------------|----------------------------------------------|
| Petrolatum primer            | 100 pounds.                                  |
| Sodium chromate inhibitor    | 1 to 1½ pounds per 100<br>pounds of primer.  |
| Potassium chromate inhibitor | 1 to 1½ pounds per 100<br>pounds of primer.  |
| Georgia clay                 | 25 to 40 pounds per 100<br>pounds of primer. |
| Polyethylene resin           | 5 pounds per 100 pounds<br>of primer.        |

said priming mass being deposited on one side of said impregnated binder for contact with objects to be protected,

and additional Georgia clay dusted on said combined covering material to facilitate separation of said roll bandage unit.

**References Cited in the file of this patent**

**UNITED STATES PATENTS**

|           |                 |                |
|-----------|-----------------|----------------|
| 2,374,565 | Roden           | Apr. 24, 1945  |
| 2,433,847 | Jennings et al. | Jan. 6, 1948   |
| 2,523,759 | Grant           | Sept. 26, 1950 |

**OTHER REFERENCES**

"Asphalts and Allied Substances" (Abraham), published by D. Van Nostrand Co., Inc. (New York), 1945 (page 533 relied on). (Copy in Div. 25.)